

1,352,710.

G. B. WATERHOUSE.  
MANUFACTURE OF STEEL.  
APPLICATION FILED JULY 31, 1919.

Patented Sept. 14, 1920.  
2 SHEETS—SHEET 1.

*Fig. 1.*



*Fig. 2.*



INVENTOR

George B. Waterhouse  
BY

J. Proc. millward.  
ATTORNEY

G. B. WATERHOUSE.  
MANUFACTURE OF STEEL.  
APPLICATION FILED JULY 31, 1919.

1,352,710.

Patented Sept. 14, 1920.

2 SHEETS—SHEET 2.

*Fig. 3.*



*Fig. 4.*



INVENTOR  
George B.  
Waterhouse  
By—

H. B. Woodward  
ATTORNEY

# UNITED STATES PATENT OFFICE.

GEORGE B. WATERHOUSE, OF BUFFALO, NEW YORK.

## MANUFACTURE OF STEEL.

1,352,710.

Specification of Letters Patent. Patented Sept. 14, 1920.

Application filed July 31, 1919. Serial No. 314,442.

To all whom it may concern:

Be it known that I, GEORGE B. WATERHOUSE, a citizen of the United States, residing at Buffalo, in the county of Erie and 5 State of New York, have invented new and useful Improvements in the Manufacture of Steel, of which the following is a specification.

This invention relates to improvements in 10 the manufacture of low and low medium carbon steels and particularly steels which are high in their sulfur content including steels particularly adapted for machining, thread cutting and drawing as extensively 15 used in the manufacture of screws, nuts and bolts in automatic cutting machines. As is well known steels as at present manufactured for use in automatic machines are characterized by high content of sulfid of 20 manganese which greatly improves the machining properties of the steel, causing the chips thereof to break off short in the machining operation.

A peculiarity of the low and low medium 25 carbon steels as produced by the methods at present employed is that there is a pronounced lack of uniformity in the distribution of the sulfur content, the latter being very irregularly distributed and forming local 30 concentrations which in the cross sectional area of the steel in a sulfur print show as peculiar spotted local growths of high sulfur material in variegated effect. In the machining of the resulting product there is 35 in consequence a corresponding irregularity in the breaking off of the chips. By the terms low medium and low carbon steel it will be understood that steels with a maximum of about .25% of carbon are contemplated and may be as low as about .04% of 40 carbon.

The improved process or method of manufacture of the present invention has for its object to produce a steel of this general character 45 which will be improved in its physical structure particularly with relation to the sulfur distribution and consists in the addition of a deoxidizer, preferably silicon in the form of ferro-silicon and desirably in the 50 ladle. I have found in practice that such addition materially improves the physical condition of the resulting steel in that substantial uniformity in the distribution of the sulfur content is obtained. In consequence 55 of the more even distribution of the sulfid the product is materially improved and

in use there will be a regular and uniform breaking off of the chips which is desirable.

In accomplishing this improvement in the physical condition of the steel by means of 60 the preferred ferro-silicon addition, such addition is proportioned to the steel being made so that the maximum silicon remaining in the steel will be but the normal requirement or normal content and necessarily may not 65 show an increase in the silicon content over that found in steels made without the silicon addition of my invention. As a result of subjecting the molten steel in the ladle to the influence of a silicon addition in accordance with my invention it has been noted that, in addition to improving the physical structure of the resulting steel by the elimination of high sulfur accumulations, there is a slight change of composition as 70 indicated by the production of a sulfo-silicid instead of a straight sulfid in the resulting steel. As the former is more brittle than the latter the resulting steel is correspondingly better adapted for automatic machining in addition to its aforesaid improvement resulting from the uniform distribution of the sulfur content.

While as described my improved process is advantageous in its application to the 85 manufacture of improved steels for machining, threading and drawing, characterized by a high sulfur content it will be understood that my improved process is also effective and valuable in obtaining improved 90 distribution of the sulfur in forging and special grade steels with a normal sulfur content. It will be further understood that the process of my invention is further instrumental in effecting a substantial improvement in the soundness and physical structure of the steel in general in addition to the sulfur distribution thereby improving the workability and rolling qualities of 95 the steel.

By way of illustration of the improvement in the sulfur distribution resulting from my improved process over that of the methods heretofore employed I have shown in the drawing herewith reproductions of 105 sulfur prints taken from bars which have been produced by the ordinary method without my improved sulfur addition and also bars produced with the sulfur addition in accordance with my invention and indicating 110 the material improvements in the distribution of the sulfur content.

In the drawings Figures 1 and 2 are facsimiles of sulfur prints taken from 2½ billets of Bessemer steel produced respectively by the customary Bessemer process and by my improved process with a ferro-silicon addition to illustrate the marked improvement in the distribution of the sulfur. Figs. 3 and 4 are similar comparative facsimiles of sulfur prints taken from blooms of open hearth steel; produced respectively by the customary process and by the process of my invention.

Referring to cross sectional area of the bar illustrated in Fig. 1, the darkened portions indicate local or concentrated areas of high sulfur material as disclosed by a sulfur print of a bar of low carbon steel produced in the usual manner without the silicon addition. Low carbon steels of this general character contain carbon up to a maximum of about 0.15% and the maximum silicon content is about 0.15% while the minimum of the latter is no increase over that found in the steels of this character without the silicon addition of my invention. The bar as illustrated in Fig. 1 is a result of the Bessemer heat which shows a ladle test analysis as follows:

|    |                      |       |      |
|----|----------------------|-------|------|
| 80 | Car                  | ----- | .13  |
|    | Man                  | ----- | .47  |
|    | Phos                 | ----- | .097 |
|    | Sul                  | ----- | .113 |
|    | Sil. in finished bar | ----- | .016 |

85 In Fig. 2 there is illustrated a bar showing substantially the same composition but produced in accordance with my improved method by being subjected to the influence of a silicon addition and is a facsimile of a sulfur print which as will be noted shows a pronounced improvement in the more uniform distribution of the sulfur and the elimination of the local growths of high sulfur material. The improved product illustrated in Fig. 2 is a result of a Bessemer heat showing an analysis as follows:

|    |                      |       |      |
|----|----------------------|-------|------|
| 50 | Car                  | ----- | .14  |
|    | Man                  | ----- | .48  |
|    | Phos                 | ----- | .097 |
|    | Sul                  | ----- | .111 |
|    | Sil. in finished bar | ----- | .016 |

In this particular instance the silicon content indicates that although subjected to the influence of the silicon addition in accordance with my invention the normal content in the product has not been increased indicating that the silicon was slagged off. In the example as shown in Fig. 2 the improved result was affected by the addition of ferro-silicon in accordance with my invention as hereinbefore described, this addition being made while the steel runs from the converter or furnace into the ladle in the preferred manner.

In Figs. 3 and 4 there is shown by comparison the material improvement in the sulfur distribution accompanying the employment of my improved process in the production of low carbon forging steels of normal 70 sulfur content. The results there indicated are facsimiles of sulfur prints taken from blooms of steel produced by the basic open hearth process in connection with which my improved process produces particularly 75 good results. The bar as illustrated in Fig. 3 was produced by the basic open hearth process in the customary manner and the darkened portions indicate the local or concentrated areas of high sulfur material and 80 is typical of its occurrence in steels of this character as ordinarily produced. The ladle test analysis of the basic open hearth heat from which the bloom of Fig. 3 was produced is as follows:

|              |       |      |
|--------------|-------|------|
| Car          | ----- | .095 |
| Man          | ----- | .46  |
| Phos         | ----- | .018 |
| Sul          | ----- | .065 |
| Sil. approx. | ----- | .02  |

85 In Fig. 4 there is shown a facsimile of a sulfur print of a bloom having substantially the same composition and produced in accordance with my invention by subjecting 95 the molten steel produced by the basic open hearth process to the influence of a ferro-silicon addition in the ladle. The product of Fig. 4 shows a ladle test analysis as follows:

|      |       |      |
|------|-------|------|
| Car  | ----- | .11  |
| Man  | ----- | .50  |
| Phos | ----- | .013 |
| Sul  | ----- | .045 |
| Sil. | ----- | .055 |

100 Thus while I have hereinbefore pointed out and shown by illustration that the process of my invention is particularly advantageous in producing Bessemer steels of improved properties it will be understood that the deoxidizing addition of my improved process may with correspondingly good results be employed in producing steels other than by the Bessemer process and is particularly effective in improving the product of the basic open hearth process. Furthermore in the preferred use of a ferro silicon addition the latter may be proportioned to vary the silicon content of the resulting steel 110 as may be desired. In this latter regard very good results have been obtained by my process wherein the resulting steel has shown no increase in the silicon content of the bar over the residual content of the 115 bath. It will be further noted that by subjecting the molten steel to the influence of the ferro-silicon addition to obtain the more uniform distribution of the sulfur content the results show that the ultimate sulfur 120

125 130 content of the steel is not increased over the 130

content in the product is unchanged or corresponds substantially to that of the untreated steel.

In so far as I am aware silicon additions have never been employed in the manufacture of low or low medium carbon steels and particularly Bessemer steels, for the purpose of bringing about the uniformity in sulfur distribution as contemplated by my improved process which as hereinbefore described successfully eliminates the variegated local growths of high sulfur material and with a material improvement in the physical structure of the resulting steel.

While I have described a preferred and particularly effective manner of carrying out the improved process of my invention it will be understood that the specific process described by way of illustration is subject to various modifications without departing from the scope of the invention as defined in the appended claims. For instance I may employ a deoxidizing addition of aluminum or aluminum and ferro-silicon but preferably I employ the ferro-silicon addition in the ladle as described.

Having described my invention, I claim:—

1. The herein described process for improving the physical structure of steels having a maximum carbon content of about .25% which consists in subjecting the molten steel to the influence of a silicon addition to effect uniformity in the sulfur distribution, said silicon addition being proportioned so as not to materially increase the silicon content of the resulting steel.

2. The herein described process for producing steels of a maximum carbon content of about .25% which consists in subjecting the molten steel to the influence of a silicon addition in the ladle to effect uniformity in the sulfur distribution, said silicon addition being proportioned so as not to materially increase the silicon content of the resulting steel.

3. The herein described process for improving the physical structure of Bessemer and basic open hearth steels of low carbon content which consists in subjecting molten steel to the influence of silicon addition to effect uniformity in the sulfur distribution, said silicon addition being proportioned so as not to materially increase the silicon content of the resulting steel.

4. The herein described process of producing low carbon steel of improved quality and having high sulfur content which consists in subjecting the molten metal to the influence of a silicon addition to effect uniformity in the sulfur distribution, said silicon addition being proportioned so as not to materially increase the silicon content of the resulting steel.

5. The herein described process for improving low carbon steels with regard to the distribution of sulfur therein which con-

sists in the addition of silicon in the ladle, substantially as described.

6. The herein described process for improving low carbon steels with regard to the distribution of sulfur therein which consists in the addition of silicon in the ladle, said silicon addition being proportioned whereby it will not materially increase the silicon content of the resulting steel.

7. The herein described process of producing low carbon steels of improved quality with regard to sulfur distribution which consists in the addition of a charge of ferro-silicon in the ladle to effect uniform distribution of the sulfur content, said addition being proportioned so as not to materially increase the silicon content of the resulting steel.

8. The herein described process of producing low medium and low carbon steels of improved quality with regard to sulfur distribution which consists in the addition of a charge of ferro-silicon in the ladle to effect uniform distribution of the sulfur content, said addition being proportioned so as not to materially increase the silicon content of the resulting steel, whereby the latter will not exceed 0.15%.

9. The herein described process for producing low carbon steels of improved quality which consists of subjecting the molten steel to the influence of a deoxidizing addition in the ladle, said deoxidizing addition consisting of ferro silicon and being proportioned so as not to materially increase the silicon content of the resulting steel and whereby the latter will not exceed 0.15%.

10. The herein described process for improving the physical structure of steels of a maximum carbon content of .25% which consists in introducing a ferro-silicon addition in the ladle to effect uniformity in the sulfur distribution.

11. The herein described process for improving the physical structure of Bessemer steels having a maximum carbon content of .25% which consists in subjecting the molten steel to the influence of a ferro silicon addition, said addition being proportioned so as not to materially increase the silicon content of the resulting steel.

12. The herein described process for improving the physical structure of Bessemer steels having a maximum carbon content of .25% which consists in subjecting the molten steel to the influence of a ferro-silicon addition in the ladle to effect uniformity in the sulfur distribution, said addition being proportioned whereby the resulting silicon content of the finished steel shall not exceed 0.15%.

In testimony whereof I have signed my name to this specification.

GEORGE B. WATERHOUSE.